

A. & M. HIRSCH.  
PROCESS OF MAKING CASTINGS OF RARE EARTH METALS AND THEIR ALLOYS.  
APPLICATION FILED MAY 9, 1918.

1,290,010.

Patented Dec. 31, 1918.

*Fig. 1.*



*Fig. 2.*



*Fig. 3.*



*Fig. 4.*



*Fig. 5.*



*Fig. 6.*



INVENTORS  
Alcan Hirsch  
Mark Hirsch  
BY  
Gorham Crosby  
ATTORNEY

# UNITED STATES PATENT OFFICE.

ALCAN HIRSCH AND MARX HIRSCH, OF NEW YORK, N. Y., ASSIGNEES TO ALPHA PRODUCTS COMPANY, INC., A CORPORATION OF NEW YORK.

## PROCESS OF MAKING CASTINGS OF RARE-EARTH METALS AND THEIR ALLOYS.

1,290,010.

Specification of Letters Patent. Patented Dec. 31, 1918.

Original application filed September 17, 1917, Serial No. 191,663. Divided and this application filed May 9, 1918. Serial No. 233,452.

To all whom it may concern:

Be it known that we, ALCAN HIRSCH and MARX HIRSCH, citizens of the United States, and residents of New York, in the county of New York and State of New York, have invented certain new and useful Improvements in Processes of Making Castings of Rare-Earth Metals and Their Alloys, of which the following is a specification.

10 The invention relates to improvements in the manufacture of castings of rare earth metals and their alloys. The improvements are particularly adapted to the manufacture of castings of alloys of cerium or lanthanum for sparking purposes. This application is a division of our prior application Serial No. 191,663 filed September 17, 1917.

Prior to the present invention it has been considered extremely difficult to cast the desired rods and shapes of cerium and its alloys having a very small cross section and volume with respect to surface, because of the extreme inflammability of the metal on the one hand and its great tendency to chemical reaction with carbon and other substances and to alloying with metals on the other hand. It was only by the laborious and wasteful process of sawing or turning beneath the surface of oil, or while constantly drenching the fresh surfaces and cuttings with oil, that it was generally known how to make the small commercial shapes necessary for use in lighters, ignition flints, etc.

35 The present process has for its object the providing of improvements whereby the rare earth metals and their alloys may be satisfactorily cast in the various forms desired in commerce and, in many cases, with sufficient exactitude of size to avoid the necessity of machining, thereby avoiding not only delay and expense, but much loss of material, which, once powdered, is extremely difficult to recover in usable shape. Also, according to the present invention, the cast metal or alloy is obtained in a most simple and economical manner and substantially free from objectionable impurities.

Further and more specific objects, features and advantages will more clearly appear from the detailed description given below taken in connection with the accompanying

sheet of drawings, which forms a part of this specification.

In the drawing,

55

Figure 1 is a vertical section of a preferred form of apparatus for melting the metals;

Fig. 2 is a top view of a mold into which the molten metal may be poured for casting; 60

Fig. 3 is a vertical section taken on the line 3—3 of Fig. 2;

Fig. 4 is a vertical section taken on the line 4—4 of Fig. 2;

Fig. 5 is a top plan view illustrating a modified form of mold; and

Fig. 6 is a similar view illustrating still another form of mold.

As an illustrative example of the improvements, the preferred process for the manufacture of castings of an alloy of cerium, lanthanum, didymium, etc., and iron will be described.

Large pigs of an alloy of cerium, lanthanum and didymium, and possibly small quantities of erbium and thorium, etc., and containing more or less impurities are broken up, as with a hammer, into pieces about one inch diameter. It is preferred to avoid using much smaller pieces than one-half inch in diameter, as they tend to thicken the melt into which they are later put, probably because of the greater amount of oxid formed on the surfaces of the pieces when an equal weight of smaller pieces is used. Larger pieces may be used, especially in the larger melts.

Into a suitable crucible, preferably a Hessian or Battersea crucible, and suitably heated, a quantity of barium chlorid crystals is put in and melted down. For this purpose, an apparatus such as shown in Fig. 1 may be used, in which 1 represents the crucible, 2 a supporting bed portion of fire-brick, provided with gas flame blasts at 3, 3, directed against the bottom part of the crucible for heating the same, 4 represents a heat insulating jacket surrounding the crucible and 5 a heat insulating cover for the crucible, and 9 a cover surrounding the top of the crucible and resting on the jacket 4. Other forms of apparatus may, however, be used.

After the barium chlorid has been fused in the crucible and the water contained in the

barium chlorid crystals has been evolved and the mass reached a quiet state of fusion, the pieces of metal, consisting mostly of cerium with some lanthanum and small quantities 5 of other metals, are washed in kerosene or other suitable oil to remove dirt, oxids and carbids that may be on the surface thereof; and then they are partially dried, as with news print paper, and then the pieces of 10 metal are added to the melt of barium chlorid in fairly large batches, that is to say, as many pieces are added at a time as can be readily shoved under the surface of the barium chlorid. Any kerosene or other 15 oil remaining on the pieces burns off as they go into the molten barium chlorid. The mass should not be stirred, and in adding the metal the melt should be agitated as little as possible. The cerium metal or alloy added 20 should preferably be low in iron, as metal high in iron not only has a higher melting point, but is apt to contain more of other impurities and these impurities are then far more difficult to separate. We, therefore, 25 prefer to use a rare earth metal containing about 10% or less of iron. When the metal added has become fluid at the bottom of the crucible, another batch of metal may be added 30 in the same way and the molten metal batch built up, care being taken not to expose the already molten cerium metal in the melt to the air, which would rapidly ignite or oxidize it. The heating of the pieces of metal to melt them should be carried out 35 relatively quickly, because, if the operation is carried out slowly, the metal melt does not become as clear and homogeneous, the fused salt above it becomes more viscous and difficult to separate from the metal, and much 40 metal is apt to be lost, nor does the metal pour so well when it is later poured from the crucible. By relatively quickly we mean that the whole operation of melting, alloying and casting the metal should take not 45 over about two hours, instead of several hours.

When the crucible is about one-half full of molten metal, as illustrated at 6 in Fig. 1, any other metal which it is desired to alloy 50 with it is added. In most cases, it is desirable to add certain other metals, such as iron, to harden the resulting alloy. This is added in the form of soft wrought iron wire. It is first cut off in pieces weighing, 55 say, 40 to 50 grams and the pieces wound into loose coils or spools. These coils of wire are poked into the melt under the layer 7 of barium chlorid. If iron alone is used, it is preferred to add sufficient iron so that the 60 resulting alloy contains about 30% of iron. The iron is preferably added periodically in about four batches. The iron becomes hot in the bath and alloys with the molten cerium, etc. The layer of barium chlorid prevents 65 oxidation of both metals. If there is

not sufficient barium chlorid in the crucible so that portions of the iron wire protrude, these portions are covered with some barium chlorid to prevent oxidation and the heating continued until they are all melted into the 70 alloy. Before the addition of any subsequent bath of iron, the previous batch of iron should be thoroughly absorbed. During the addition of the iron, care should be taken not to stir the batch any more than 75 is absolutely necessary. When all the iron or other metal is added, the temperature may be raised to about 1000° C. which increases the fluidity of the molten metal. When the melt is fairly liquid, and about 80 ten minutes before it is poured out, it is thoroughly but gently stirred to produce a homogeneous mass. It is important to increase the fluidity in order that, when stirred it shall be thoroughly mixed, and when 85 poured into the molds the molten metal will be sufficiently fluid not to be congealed prematurely as more clearly pointed out herein-after. An additional layer of barium chlorid may be added, if necessary. 90

When the metal is thoroughly molten and homogeneous, the crucible is lifted out of the furnace and a hole poked through the crust, if any, of barium chlorid adjacent the side of the crucible, by means of a hot iron 95 bar or rod. The molten metal is then poured through this hole out into suitable molds. It is desirable to make up melts of metal of over 350 grams, preferably about 2-3 kilograms, as, if smaller melts, say of 200 100 grams, are used, difficulty is encountered in pouring the metal.

While any form of molds may be used, it is preferred to make them of iron or have the casting face of iron or the like. However, graphite and other materials may be used for the molds. The mold, especially if made of solid iron, should be uniformly heated to about 400° C. It should be over 100° C. This heating of the mold permits 110 the pouring of the metal at a temperature so near to the solidifying point that excessive burning is avoided and at the same time permits this metal, near to the point of congelation, to find its way into and fill the mold. 115 The mold should be slowly and uniformly heated to prevent warping thereof. By thus heating the metal mold the residual heat absorbing capacity of the mold, up to the temperature of congelation of the molten metal 120 is reduced to a point where it does not materially affect the homogeneity of the resulting casting by causing cracks, breaks, strings and "cold shots" and similar imperfections in the casting, caused by rapid and uneven 125 cooling of the molten metal. This may be accomplished in other ways. Instead of heating a heavy metal mold a thin sheet metal mold having little heat absorbing capacity may be used to accomplish the same 130

result. In Figs. 2, 3 and 4 there is illustrated an iron mold composed of two parts 10 and 11, the part 10 being a flat iron plate, and the part 11 being a flat iron plate, provided with grooves 12, extending from the top nearly to the bottom thereof. A connecting groove 13 is provided at the top. The plates may be held together by four angle bars 14 running along near the top and bottom on the outside of the plates and pulled together by bolts 15. The resulting castings have an unusually small diameter or cross section and relatively great length and the ratio of the area in square inches of the molding surface from which withdrawal of heat may take place, to the volume in cubic inches of the casting to be produced, is greater than 16 to 1. In order that this relatively large heat withdrawal surface may 10 not cause premature congelation in the mold of the metal, already near the point of congelation, and prevent the complete flow of molten metal near the temperature of incipient congelation, into the mold, the chilling 20 capacity of the mold is reduced as above described, and the fluidity of the molten metal is increased prior to pouring, by stirring and by a slight increase in the temperature thereof, as above described, to permit the molten 30 metal to penetrate the mold cavities with substantial completeness before the stage of incipient congelation is passed.

Before pouring the metal into the mold, the surfaces of the mold may be dusted or otherwise coated with a layer of magnesia or other inert material such as rolling scale or tin plating, so that the pieces of cast metal may be easily removed from the mold. The metal is poured into the connecting slot 13 and runs into the mold slots 12, filling them up. The mold should be allowed to cool slowly, that is, no artificial means are used to hasten the cooling, but the mold is allowed to air cool, so that it cools with sufficient rapidity to prevent any substantial oxidation of the metal. If the coating of magnesia has been uniform, a slight tapping of the plate 11, after plate 10 has been removed therefrom, should so loosen the pieces of cast 50 metal that they may be easily removed.

In Fig. 5 is shown a top view of a similar mold adapted to form cylindrical-shaped castings or sticks of metal, and in Fig. 6 is shown a top view of a similar mold adapted 55 to cast sticks of metal rectangular in cross-section.

The resulting cast sticks of metal as they come from the molds shown in Figs. 2 to 6 are especially adapted for sparking purposes 60 and differ materially from the pieces of alloy heretofore used for this purpose and which were made by sawing or turning under oil. The alloy castings made according to our process, have matt unsmeared glassy surfaces 65 where formed adjacent the metal mold

surface. While the surfaces may be somewhat rough owing to the presence of some air or blow holes on the surface, yet the surfaces have a characteristic glassy appearance and the metal is not smeared over as is the case when the pieces are formed by sawing or turning. Moreover, especially when cast in the metal molds, it is found that the castings at said surfaces have a superficial skin 70 partly composed of the alloy, but poorer in the rare earth metal than is the alloy in the interior of the cast piece. This probably is due to the alloy taking up metal or particles from the metal mold surface. This skin serves as a substantially non-corrosive coating or layer while the necessary sparking properties are not interfered with thereby. By melting and pouring the alloyed metals from beneath a fused salt as above described, flakes of oxid, which would otherwise be 85 present in the casting, are substantially eliminated and the resultant casting is extremely homogeneous.

In many cases, it is found that crude metal (chiefly cerium or lanthanum), as taken 90 from the electrolytic cell in which it is produced, is so impure or non-homogeneous that a stable and sufficiently air-resistant alloy is not produced by a single fusion of the crude metal under the purifying bath. 95 as of barium chlorid. In such case, it is desirable to make two or more successive fusions as described, preferably before alloying (raising the melting point) and casting into final shapes (separating the metal or 100 alloy into small pieces). After each such preliminary purifying fusion, the slag or fused salt may be removed from the crucible and fresh purifying salt already dehydrated added to the metal therein, or the 105 metal may be cast into pigs of convenient size (about 1x1x4 inches) for remolding or for breaking into lumps for remelting.

While it has been suggested that in the making of certain brass, bronze and steel 110 alloys, the metal may be melted below a layer of borax or waterglass, this is a very different proposition from the making of castings of the rare earth metals, such as cerium or lanthanum, and their pyrophoric 115 alloys which congeal readily and pour with difficulty near their congealing point. Cerium is not only readily oxidized when heated, but rapidly ignites, and, furthermore, has such a great affinity for oxygen 120 that if melted below such glass as borax or waterglass, would so rapidly combine with the oxygen therein as to cause a violent reaction. With the brass, bronze and steel 125 alloys, there is no such problem. The making of bronze, brass and steel castings is an art distinct and separate from the art of making castings and suitable for commercial use from pyrophoric alloys of cerium and similar rare earth metals in which the 130

metals are so chemically active that they even unite readily with carbon to form carbide.

- 5 It has also been suggested that alloys can be prepared by melting together certain quantities of a rare earth metal and aluminum under a covering layer of sodium chlorid and potassium chlorid, but unless certain additional features or precautions are employed in the process, the results are very unsatisfactory and even then barium chlorid has distinct advantages not possessed by a mixture of sodium chlorid and potassium chlorid.
- 10 15 Instead of using barium chlorid as a protecting layer for the molten metal, sodium chlorid and other salts inert to the rare earth metal being used, may be used which would prevent oxidation of the metal, but barium chlorid has advantages over certain other salts, because of its less volatility at the working temperature. If more volatile salts are used, there is not only a corresponding loss of the salt, but great inconvenience to the workmen results. Furthermore, it is believed that the surface tension of fused cerium and its alloys against a molten bath high in barium chlorid is far more advantageous to making homogeneous castings and protecting the surface of the metal from too rapid oxidation. Copper or magnesium may also be added to the molten metal to harden the resulting alloy, or increase the fatness and heat of the spark.
- 20 25 30 35 30 Other methods preventing oxidation of the melt may be used as by carrying out the fusion in an atmosphere of hydrogen.

Many other changes and modifications may be made without departing from the spirit and scope of the invention in its broader aspects.

What is claimed as new and desired to be secured by Letters Patent is:—

1. In the process of making castings of cerium and similar rare earth metals and their alloys, the steps which consist in melting the rare earth metal and pouring it into molds, the temperature of the metal when poured being sufficiently close to the congelation temperature to prevent inflammation of the metal.
- 45 50 55 60 65 2. In the process of making casting of cerium and similar rare earth metals and their alloys, the step which consists in pouring the molten rare earth metal or alloy thereof into a mold with a metal molding surface in which the ratio of the area in square inches, of the molding surface from which withdrawal of heat may take place, to the volume in cubic inches of the casting produced, is greater than 16 to 1, the residual heat absorbing capacity of the mold, up to the temperature of congelation of the molten metal, being reduced to a point where it does not materially affect the homogeneity

of the resulting casting by imperfections in the casting caused by rapid and uneven cooling of the molten metal.

3. In the process of making castings of alloys of cerium or lanthanum the steps which consist in melting rare earth metal containing mainly cerium or lanthanum and protecting the molten metal from oxidation and pouring the molten metal into molds heated to about 100° C. or over.

75 4. In the process of making castings of alloys of cerium or lanthanum the steps which consist in melting rare earth metal containing mainly cerium or lanthanum and protecting the molten metal from oxidation and pouring the molten metal into molds and allowing the molds to cool slowly as at room temperature, the residual heat absorbing capacity of the mold, up to the temperature of congelation of the molten metal, being reduced to a point where it does not materially affect the homogeneity of the resulting castings by imperfections in the casting caused by rapid and uneven cooling of the molten metal.

90 5. In the process of making castings of cerium and similar rare earth metals and alloys thereof, the steps which consist in melting the rare earth metal or alloy thereof while protecting the molten metal from oxidation, pouring the molten metal into molds, the temperature of the metal when poured being sufficiently close to the congelation temperature to prevent inflammation of the rare earth metal, and permitting the metal to cool in the mold, with sufficient rapidity to prevent any substantial oxidation thereof.

95 6. In the process of making castings of cerium and similar rare earth metals and their alloys the steps which consist in melting the rare earth metal and pouring the molten metal into molds heated to about 100° C. or over.

100 110 115 7. In the process of making castings of cerium and similar rare earth metals and their alloys the steps which consist in melting the rare earth metal and pouring the molten metal into molds heated to about 100° C. or over, and allowing the molds to cool slowly as to room temperature, the molds being coated with finely divided inert material to render the cast metal more easily removable therefrom.

120 125 8. In the process of making castings of cerium and similar rare earth metals and their alloys the steps which consist in melting a rare earth metal while protecting the molten metal from oxidation, and pouring the molten metal into molds, the whole operation taking about two hours or less, the residual heat absorbing capacity of the mold, up to the temperature of congelation of the molten metal, being reduced to a point where it does not materially affect the ho- 130

mogeneity of the resulting castings by imperfections in the casting caused by rapid and uneven cooling of the molten metal.

9. In the process of making castings of cerium or similar rare earth metals or alloys thereof the steps which consist in melting rare earth metal containing mainly cerium or lanthanum and containing about 10% or less of iron, and then melting therewith an alloying metal to harden the resulting alloy, and pouring the molten rare earth metal or alloy thereof into a mold with a metal molding surface in which the ratio of the area in square inches, of the molding surface from which withdrawal of heat may take place, to the volume in cubic inches, of the casting produced is greater than 16 to 1, the residual heat absorbing capacity of the mold, up to the temperature of congelation of the molten metal, being reduced to a point where it does not materially affect the homogeneity of the resulting casting by imperfections in the casting caused by rapid and uneven cooling of the molten metal.
10. In the process of making castings of cerium or similar rare earth metals or alloys thereof the steps which consist in melting rare earth metal containing mainly cerium or lanthanum containing less than about 10% of iron and pouring the molten rare earth metal or alloy thereof into a mold with a metal molding surface in which the ratio of the area in square inches, of the molding surface from which withdrawal of heat may take place, to the volume in cubic inches, of the casting produced, is greater than 16 to 1, the residual heat absorbing capacity of the mold, up to the temperature of congelation of the molten metal, having been reduced to a point where it does not materially affect

the homogeneity of the resulting casting by imperfections in the casting caused by rapid and uneven cooling of the molten metal.

11. In the process of manufacturing castings of rare earth metal alloys the steps which consist in pouring the molten alloy, at a temperature near the temperature of incipient congelation thereof, into multiple molds, the mold cavities of which have a surface to volume ratio measured in square inches and cubic inches respectively, greater than 16 to 1; and reducing the heat abstracting capacity of the molding surface to such a point that the molten metal penetrates the mold cavities with substantial completeness before the stage of incipient congelation is passed.

12. In the process of manufacturing castings of cerium and similar rare earth metals or their alloys, the steps which consist in melting the rare earth metal or alloy and pouring the molten metal into molds, the residual heat absorbing capacity of which, up to the temperature of congelation of the molten metal, is reduced to a point where it does not affect the homogeneity of the resulting casting by imperfections in the casting caused by rapid and uneven cooling of the molten metal and permitting the metal to cool in the mold with sufficient rapidity to prevent any substantial oxidation thereof.

Signed at New York, in the county of New York and State of New York, this 6th day of May, A. D. 1918.

ALCAN HIRSCH.  
MARX HIRSCH.

Witnesses:

J. R. BAILEY,  
R. G. TRIMBLE.